# EUROPEAN PATENT SPECIFICATION

(11) **EP 0 116 216 B1**
(45) Date of publication and mention of the grant of the patent: **26.03.1986**
(21) Application number: 83307543.5
(22) Date of filing: 12.12.1983
(51) Int. Cl.: D01G 1/10, B68G 3/00, B68G 7/06

(54) **Process for the manufacture of filling fibres**
Verfahren zur Herstellung von Füllfasern
Procédé de production des fibres de rembourrage

(30) Priority: 12.01.1983 GB 8300771
(43) Date of publication of application: 22.08.1984
(73) Proprietor: IMPERIAL CHEMICAL INDUSTRIES PLC, London SW1P 3JF (GB)
(72) Inventor: Davidson, Alistair J., Harrogate North Yorkshire (GB)
(74) Representative: Corbett, William Michael

## Description

This invention relates to a process for the manufacture of a filling material for articles such as quilts, pillows, and clothing.

In recent years, considerable development has been made in the use of man-made fibres as a replacement for natural material, such as feathers and down, as filling material for quilts, pillows, and clothing, and other similar articles. One way in which man-made fibres are used for this purpose is to take the crimped, staple fibres which are sold by the fibre manufacturers, in the form of a compressed bale, and to blow the fibres by means of a stream of compressed air into the article to be filled. To work satisfactorily, it is necessary for the staple fibres on removal from the bale to be opened by a mechanical means, such as by passing the fibres through a carding machine. (DE-A-2702166) carding machines' are rather complex and expensive, and for satisfactory operation require to be run continuously rather than intermittently.

We have now found that it is possible to produce staple fibres for blow filling articles by a cheaper and more convenient route using a "threaded roll module".

According to the present invention there is provided a process for the blowfilling of an article with staple filling fibres, the process comprising the steps in sequence of de-registering the filaments of at least one tow of crimped continuous fibres by passage through a threaded roll module, as hereinafter defined, cutting the deregistered tow into staple fibres, and blowing the cut fibres into the article to be filled.

By the term "threaded roll module" is meant a machine comprising at least one pair of rolls, the surface of at least one of which is made up of grooves and ridges, the grooves encircling the roll in the form of one or more helices or a large number of parallel and endless grooves, so that when a tow of filaments is passed between a pair of rolls the filaments are only gripped between the rolls at the ridges and little or no grip is applied to the remaining filaments. As the rolls rotate, different filaments are gripped and released, and are caused to undergo lateral movement relative to other filaments.

Preferably, a threaded roll module comprises successive pairs of rolls, the periferal speed of a pair of rolls being greater than that of the preceding pair of rolls, but insufficiently fast to put the tow under substantial tension, so that the crimp in the filaments is noticeable even between roll pairs, while the tow is deflected out of its normal running path with ease. The threaded roll module is described in considerable detail in British Patent Specification No. 1 001 813.

Tow of crimped fibres suitable for use in the process of the present invention is that supplied by fibre manufacturers specifically for processing through a threaded roll module for the manufacture of filling material comprising continuous filaments.

The deregistered tow of continuous filaments may be cut into staple fibre by passage through any convenient cutter, such as that made by Lummus Industries Inc. The cut fibre may be blown into an article to be filled by any conventional equipment.

Advantageously, the three steps of the process of the present invention are operated without a break in which case the threaded roll module, cutter, and blower for the cut fibre are operated sequentially in-line, and consequently by a single operative. In this way, the equipment may be operated intermittently, providing cut staple filling fibres as and when required for blow filling an article. Alternatively one or two steps of the process may be operated at a different time or even a different location from the others if necessary. For instance the tow of continuous fibres may be deregistered by passage through a threaded roll module and cut into staple fibres at one location, and transferred to another location where the cut fibre is blown into an article to be filled.

Further advantages of the process of the present invention over the conventional process are superior opening of the fibre, higher throughput, and the capability of satisfactorily processing blends of fibres of different decitex, different cross-section, different crimp levels or formed from different 'polymers.

The present invention is further illustrated by the following example.

### Example 1

A tow of 33 K tex hollow poly(ethylene terephthalate) filaments each of 4.4 decitex was opened by a passage through a threaded roll module comprising two pairs of rolls, generally as described in British Patent No. 1 001 813. The fibres where then cut into lengths of 26 mm by a conventional staple cutter made by Lummus Industries Inc, and then blown into a quilt using conventional equipment designed for the blow filling of feathers and down.

## Claims

1. A process for the blow filling of an article with staple filling fibres characterised in that it contains the steps in sequence of deregistering the filaments of at least one tow of crimped continuous fibres by passage through a machine comprising at least one pair of rolls, the surface of at least one of which is made up of grooves and ridges, the grooves encircling the roll in the form of one or more helices or a large number of parallel and endless grooves, so that when a tow of filaments is passed between a pair of rolls the filaments are only gripped between the rolls at the ridges and little or no grip is applied to the remaining filaments, cutting the deregistered tow .into staple fibres, and blowing the cut fibres into the article to be filled.

2. A process according to claim 1 wherein there is a break between one or more of the steps.

## Patentansprüche

1. Verfahren zum Füllen eines Gegenstands durch Einblasen von Stapelfasern, gekennzeichnet durch die nachstehende Abfolge von Stufen: Außberphasebringen der Filamente mindestens eines Kabels aus gekräuselten kontinuierlichen Fasern durch Hindurchführen durch eine Maschine, die mindestens ein Rollenpaar aufweist, wobei zumindest eine Oberfläche derselben mit Nuten und Rippen versehen ist, welche Nuten die Rolle in Form ein oder mehrerer Schraubenlinien oder in Form einer großen Anzahl von parallelen und endlosen Nuten umgeben, so daß, wenn ein Kabel aus Filamenten zwischen ein Rollanpaar hindurchgeführt wird, die Filamente zwischen den Rollen nur an den Rippen ergriffen werden und die übrigen Filamente nur wenig oder gar nicht ergriffen werden, Schneiden des außer Phase gebrachten Kabels in Stapelfasern und Einblasen der geschnittenen Fasern in den zu füllenden Gegenstand.

2. Verfahren nach Anspruch 1, bei welchem nach einer oder mehreren Stufen eine Unterbrechung erfolgt.

## Revendications

1. Procédé pour le rembourrage par soufflage d'un article au moyen de fibres de rembourrage coupées, caractérisé en ce que, successivement, on dérange les filaments d'au moins un faisceau de fibres continues crêpées par passage à travers une machine comprenant au moins une paire de rouleaux, la surface d'au moins un des rouleaux présentant des gorges et des nervures, et les gorges encerclant le rouleau sous la forme d'une ou de plusieurs hélices ou d'un grand nombre de gorges parallèles et sans fin, de sorte que lorsqu'un faisceau de filaments est passé entre les rouleaux d'une paire, les filaments ne soient pris entre les rouleaux qu'au niveau des nervures et que la prise exercée sur les filaments restants soit faible ou nulle, on sectionne le faisceau dérangés en fibres coupées et on souffle les fibres coupées dans l'article à rembourrer.

2. Procédé suivant la revendication 1, dans lequel une interruption est prévue après une ou plusieurs des opérations.
